

# United States Patent Office

3,556,797

Patented Jan. 19, 1971

1

3,556,797

**COBALT (II) AND MANGANESE (II) CHELATES AS  
PHOTOGRAPHIC EMULSION ANTIFOGGANTS**  
Hendrik Adolf Pattijn, Wilrijk, Robrecht Julius Thiers,  
Brasschaat, Bernard Hippoliet Tavernier, Edegem, and  
Jozef Frans Willems, Wilrijk, Belgium, assignors to  
Gevaert-Agfa N.V., Mortsel, Belgium, a company of  
Belgium

Belgium  
No Drawing. Filed Apr. 19, 1968, Ser. No. 722,558  
Claims priority, application Great Britain, May 18, 1967  
23,048/67; Oct. 19, 1967, 47,731/67

23,048/67; Oct. 19, 1967, 47,731/67  
Int. Cl. G03c 1/34

U.S. Cl. 96—109

U.S. Cl. 96—109 8 Claims

## ABSTRACT OF THE DISCLOSURE

Photographic light-sensitive silver halide emulsions are described which include a cobalt (II) or a manganese (II) chelate of a (poly) amino-(poly)carboxylic acid in acid form or in the form of a water-soluble salt. These materials exert an excellent stabilizing and fog-inhibiting action upon the photographic light-sensitive materials.

This invention relates to fog-inhibiting agents and stabilizers for photographic light-sensitive silver halide emulsions and to photographic emulsions containing them.

Light-sensitive silver halide emulsions are in general characterised by their sensitivity, gradation and fog.

As is well-known, sensitivity, gradation and fog are determined by the way in which the silver halide emulsion is prepared and by the use of special chemical ingredients effecting a desired improvement or result. Addenda to the emulsion, which are of particular importance for the stability of the light-sensitive characteristics of a silver halide emulsion are the so-called "stabilizers."

Stabilizers or antifoggants protect the light-sensitive silver halide emulsions against spontaneous formation and growth of fog known as chemical fog during prolonged storage or storage at high temperatures and humidities or during development to maximum contrast and speed, or both. Indeed, the fog increases with the degree and temperature of development, and, in constant development circumstances, with the time the light-sensitive emulsion is stored and with the temperature and the relative humidity of the atmosphere wherein the emulsion is stored. It is evident that a light-sensitive emulsion should be obtained which is as stable as possible at high temperature and high relative humidity for instance in view of its use in tropical countries.

It is known to protect light-sensitive silver halide emulsions against the growth of chemical fog during storage by addition of stabilizers of the triazolopyrimidine type (azaindolizines). However, emulsions stabilized with compounds of the triazolopyrimidine type still show a tendency to fog formation in extreme storage circumstances i.e. at very high temperatures and humidities and in extreme development circumstances e.g. rapid processing at elevated temperatures.

It is also known to use heterocyclic thioxo and mercapto compounds as stabilizers for photographic silver halide emulsions but these compounds generally show the disadvantage of impairing the sensitivity and gradation.

From United States Pat. 2,839,405 it is known that certain water-soluble inorganic acid salts, more particularly inorganic acid salts of cadmium, cobalt, manganese and zinc, are effective for inhibiting fog and stabilizing silver halide emulsions during incubation.

It has now been found that when incorporating in a light-sensitive material comprising a silver halide emul-

2

sion layer cobalt (II) and manganese (II) chelates of (poly)amino-(poly)-carboxylic acids, in acid form or in the form of a water-soluble salt, these compounds exert a stabilizing and fog-inhibiting action upon said photographic light-sensitive material exceeding that of the simple inorganic acid salts of cobalt and manganese referred to above without causing an appreciable desensitization of said material.

Moreover, it has been found that these cobalt (II) and manganese (II) chelates are very suitable for use in combination with stabilizers of the triazolopyrimidine type, particularly in extreme storage and development circumstances in order to reduce the fogging tendency of the light-sensitive emulsion.

15 The cobalt (II) and manganese (II) chelates of (poly)-  
amino-(poly)carboxylic acids can be prepared in a very  
simple way, namely by allowing to react a water-soluble  
cobalt (II) or manganese (II) salt (chloride, acetate,  
nitrate, sulfate, etc.) with a (poly)amino-(poly)carboxylic  
20 acid sequestering compound or water-soluble salt there-  
of.

25 Examples of suitable (poly)amino-(poly)carboxylic acid sequestering compounds for reaction with a cobalt (II) or manganese (II) salt to form the corresponding cobalt (II) and manganese (II) chelates as well as details about the preparation of said sequestering compounds can be found in Ind. Chim. Belg. Tome XXI (1956) pp. 338-346 and in Ind. Chim. Belg. Tome XXIII (1958) pp. 1105-1115.

30 Particularly suitable (poly)amino-(poly)carboxylic acids for forming in acid or salt form with a cobalt (II) or manganese (II) salt the corresponding cobalt (II) or manganese (II) chelates can be represented by the following non-limitative general formula:



wherein:

L stands for alkylene including substituted alkylene e.g. hydroxylalkylene, cycloalkylene including substituted cycloalkylene or alkylene interrupted by one or more hetero atoms, such as an oxygen atom,

$x$  represents 0, 1 or 2,  
 R stands for lower alkylene e.g. methylene and ethylene including substituted lower alkylene e.g. alkylene substituted by alkyl, aryl, aralkyl, including substituted alkyl, aryl and aralkyl, and each of  $R_1$  and  $R_2$  (the same or different) stands for hydrogen, lower alkyl including substituted lower alkyl, aralkyl including substituted aralkyl or aryl including substituted aryl; examples of substituted alkyl groups for  $R_1$  and for  $R_2$  are alkyl substituted with hydroxyl, halogen, alkoxy, carbamoyl, amino, substituted amino e.g. dihydroxyalkylamino, epoxy, carboxyl, sulfo, phosphono, mercapto, alkyl-mercapto, alkoxy carbonyl, a nitrogen-containing heterocyclic ring e.g. pyridyl and examples of substituted aryl groups and aralkyl groups for  $R_1$  and/or  $R_2$  are: aryl and aralkyl substituted by hydroxyl, halogen, alkyl, alkoxy, nitro, carboxyl and sulfo.

65 The following is a non-limitative list of examples of (poly)amino(poly)carboxylic acids corresponding to the above general formula:



- (2)   
1,2-propylenediamine, N,N,N',N'-tetraacetic acid
- (3)   
ethylenediamine, N,N,N',N'-tetrapropionic acid
- (4)   
N-(2-hydroxyethyl)-ethylenediamine, N,N',N'-triacetic acid
- (15)   
ethyleneglycol bis(2-aminoethyl)-N,N,N',N'-tetraacetic acid
- (5)   
N-(2-hydroxypropyl)-ethylenediamine, N,N',N'-triacetic acid
- (6)   
N-(2,3-dihydroxypropyl)-ethylenediamine, N,N',N'-triacetic acid
- (7)   
N,N'-di(2-hydroxyethyl)-ethylenediamine, N,N'-diacetic acid
- (8)   
diethylenetriamine, N,N,N',N'',N'''-pentaacetic acid
- (9)   
nitrilo triacetic acid
- (10)   
ethylenediamine, N,N'-di-(o-hydroxyphenyl) acetic acid
- (11)   
di(2-hydroxyethyl)-amino acetic acid
- (12)   
2-hydroxyethyl-amino diacetic acid

- (13)   
1,2-aminocyclohexane, N,N,N',N'-tetraacetic acid
- (14)   
2,3-dihydroxypropyl-aminodiacetic acid
- (16)   
N,N'-di[3-di(2-hydroxyethyl)amino-2-hydroxy-propyl]-ethylenediamine, N,N'-diacetic acid
- (17)   
N-(2-hydroxyethyl)-N'-(a-pyridinomethyl)-ethylenediamine, N,N'-diacetic acid
- (18)   
N-(2-hydroxyethyl)-N'-phosphonomethyl-ethylenediamine, N,N'-diacetic acid
- (19)   
N-(2,3-dihydroxypropyl)-N'-(2-sulphoethyl)-ethylenediamine, N,N'-diacetic acid
- (20)   
N,N'-di(2-hydroxyethyl)ethylenetriamine, N,N',N'''-triacetic acid
- (21)   
N-(2-mercaptop-1-carboxy-ethyl)-N'-(2-hydroxyethyl)-ethylenediamine, N,N'-diacetic acid
- (22)   
N-(3,5-dichloro-4-hydroxy-benzyl)-N'-(2-hydroxy-ethyl)-ethylenediamine, N,N'-diacetic acid
- (23)   
2-hydroxy-propylene diamine, N,N,N',N'-tetraacetic acid
- (15)   
5
- (10)   
10
- (14)   
14
- (30)   
30
- (40)   
40
- (45)   
45
- (50)   
50
- (55)   
55
- (60)   
60
- (65)   
65
- (70)   
70
- (75)   
75

As compared with the known cobalt and manganese compounds used as stabilizers the cobalt (II) and manganese (II) chelates according to the present invention when used in the appropriate concentration have a markedly better fog-inhibiting action.

The antifoggants according to the present invention are particularly suitable for use in conjunction with compounds which sensitize the emulsion by development acceleration for example alkylene oxide polymers. These alkylene oxide polymers may be of various type. Various derivatives of alkylene oxides may be used to sensitize the silver halide emulsions e.g. alkylene oxide condensation products as described among others in United States Pats. 2,531,832 and 2,533,990, in United Kingdom patent specifications 920,637, 940,051 945,340 and 991,608 and in Belgian patent specification 648,710. Other compounds that sensitize the emulsion by development acceleration and that are suitable for use in combination with the cobalt (II) and manganese (II) chelates of the invention are the onium derivatives of amino-N-oxides as described in the published Dutch patent application 6612269.

The stabilizers according to the invention can also be used in conjunction with other known stabilizers for instance with heterocyclic nitrogen containing thioxo compounds such as benzothiazoline - 2 - thione and 1-phenyl-2-tetrazoline-5-thione, with mercury compounds such as those described in Belgian patent specifications 524,121 and 677,337 and in the published Dutch patent application 6715932 and, as said above, preferably with compounds of the hydroxytriazolopyrimidine type (azaindolizines).

The stabilizers according to the present invention may be incorporated into any type of light-sensitive material comprising a silver halide emulsion layer, e.g. a spectrally sensitized or non-sensitized silver halide emulsion layer, a silver halide emulsion layer of use in diffusion transfer processes for the production of silver images, an X-ray emulsion layer, and an emulsion layer sensitive to infrared radiation. They may be incorporated into high-speed negative materials as well as into rather low speed positive materials. Various silver salts may be used as light-sensitive salt e.g. silver bromide, silver iodide, silver chloride, or mixed silver halides e.g. silver chloro-bromide or silver bromo-iodine.

The silver halides are dispersed in the common hydrophilic colloids such as gelatin, casein, zein, polyvinyl alcohol, carboxymethylcellulose, alginic acid, etc., gelatin being however favoured.

The stabilizing agents are generally incorporated into the silver halide emulsion layer of the light-sensitive material; they may be added to the emulsion during any step of emulsion preparation; however, they are preferably added to the photographic emulsion after chemical ripening and just before coating of the emulsion. The addenda according to the present invention are incorporated into the photographic emulsions according to the methods well known in emulsion preparation, e.g. in the form of a solution in any convenient solvent not injurious to the emulsion such as water or lower alcohols.

Instead of incorporating the compounds of the invention into the emulsion layer they can also be incorporated into another layer of the photographic material, e.g. a gelatin antistress layer or intermediate layer, which is in water-permeable relationship with the said emulsion layer.

The amount of cobalt (II) and manganese (II) chelate employed in the light-sensitive silver halide material depends on the particular type of emulsion and the desired effect and can vary within very wide limits. The optimum amount of cobalt (II) and manganese (II) chelate to be added can be determined for each particular type of emulsion in a very simple way by application of the usual tests. Usually said compounds are employed in a ratio of about 0.1 g. to about 20 g. per mole of silver

halide, preferably from 0.5 to 10 g. per mole of silver halide, when incorporated into the emulsion layer itself and in an amount of about 10 mg to 1 g. per sq. m. when incorporated into a layer in water-permeable relationship with the emulsion layer.

The light-sensitive emulsions may be chemically as well as optically sensitized. They may be chemically sensitized by effecting the ripening in the presence of small amounts of sulfur containing compounds such as allyl-thiocyanate, allyl thiourea, sodium thiosulfate, etc. The emulsions may also be sensitized by means of reducers for instance tin compounds as described in our French patent specification 1,146,955 and in our Belgian patent specification 568,687, imino-amino methane sulfonic acid compounds as described in our United Kingdom patent specification 789,823 and small amounts of noble metal compounds such as of gold, platinum, palladium, iridium, ruthenium and rhodium.

Other addenda such as hardening agents, wetting agents, plasticizers, color couplers, developing agents and optical sensitizers can be incorporated into the emulsion in the usual way.

The following examples illustrate the present invention.

#### EXAMPLE 1

A gelatino silver bromoiodide emulsion (2 mole percent of iodide) comprising 400 mg. per mole of silver halide of 5-methyl-7-hydroxy-s-triazolo - [1,5-a] - pyrimidine as stabilizer, and 1 g. per litre of emulsion of saponin as coating aid, was prepared in the conventional manner and then divided into 2 aliquot portions.

To emulsion portion B were added 5.5 g. per mole of silver halide of the cobalt (II) chelate of compound 1 disodium salt, whereas to emulsion portion A no cobalt (II) chelate was added.

The two emulsions were coated on both sides of a subbed cellulose triacetate support in such a way that an amount of silver halide equivalent to 10 g. of sq. m. of silver nitrate was present. The emulsion layers were then overcoated with a gelatin antistress layer.

Strips of the two materials thus obtained were stored for 36 hours in an atmosphere of 57° C. and 35% relative humidity.

The stored material strips as well as strips of the freshly prepared materials were exposed and developed for 8 minutes at 20° C. in a developing bath with the following composition:

Water—800 ccs.  
p-Monomethylaminophenol sulphate—4 g.  
Sodium sulfite (cryst.)—130 g.  
Hydroquinone—10 g.  
Sodium carbonate (cryst.)—120 g.  
Potassium bromide—5 g.  
Water to make, 1000 ccs.

After the treatment in a stop bath, rinsing and fixing of the material strips the following sensitometric results were attained.

| 60 | Freshly prepared |      |           | Stored for 26 hrs. at 57° C./<br>35% RH |      |           |                         |
|----|------------------|------|-----------|-----------------------------------------|------|-----------|-------------------------|
|    | Material         | Fog  | Gradation | Relative speed, percent                 | Fog  | Gradation | Relative speed, percent |
| 65 | A-----           | 0.10 | 2.60      | 100                                     | 1.14 | 2.50      | 107                     |
|    | B-----           | 0.08 | 2.80      | 89                                      | 0.07 | 2.80      | 98                      |

#### EXAMPLE 2

A gelatino silver bromoiodide emulsion was prepared as described in Example 1 and divided into three aliquot portions.

Each of the three emulsion portions was coated on both sides of a subbed cellulose triacetate support, in such a way that on both sides an amount of silver halide equivalent to 8 g. of silver nitrate was present per sq. m., and

dried. The emulsion layers of the three materials A, B and C were then overcoated with a gelatin antistress layer, the antistress layers of materials B and C containing 0.07 and 0.28 g. per sq. m. respectively of the cobalt (II) chelate of compound 1 disodium salt.

Strips of the three materials were conditioned in a moist atmosphere of about 75% relative humidity and then packed in aluminum-laminated paper and finally stored for 1 week at 59° C. Other strips were stored for 36 hours in an atmosphere of 57° C. and 34% relative humidity.

The stored material strips as well as strips of the freshly prepared materials were further treated as described in Example 1.

The following sensitometric results were attained.

| Material | Freshly prepared |           |                     | Stored for 36 hrs. at 57° C./34% RH |           |                     | Stored for 1 week at 59° C./75% RH |           |                     |
|----------|------------------|-----------|---------------------|-------------------------------------|-----------|---------------------|------------------------------------|-----------|---------------------|
|          | Fog              | Gradation | Rel. speed, percent | Fog                                 | Gradation | Rel. speed, percent | Fog                                | Gradation | Rel. speed, percent |
| A        | 0.09             | 2.43      | 100                 | 0.12                                | 2.18      | 100                 | 0.24                               | 2.60      | 104                 |
| B        | 0.08             | 2.45      | 98                  | 0.08                                | 2.33      | 98                  | 0.10                               | 3.00      | 98                  |
| C        | 0.08             | 2.53      | 91                  | 0.08                                | 2.44      | 2.44                | 0.10                               | 3.15      | 91                  |

### EXAMPLE 3

A gelatino silver bromoiodide emulsion (2 mole percent of iodide) was prepared and divided into five aliquot portions.

Each of the five emulsion portions was coated on a subbed cellulose triacetate support, in such a way that on both sides an amount of silver halide equivalent to 8 g. per sq. m. of silver nitrate was present, and dried. The emulsion layers of the five materials A, B, C, D and E were then overcoated with a gelatin antistress layer proportion of 1 g. of gelatin per sq. m. The gelatin antistress layers of material B comprised, on each side, 250 mg. per sq. m. of the cobalt (II) chelate of compound 1 disodium salt, whereas the gelatin antistress layers of materials C, D and E comprised equivalent amounts per sq. m. of cobalt (II) sulfate, cobalt (II) acetate and cobalt (II) chloride respectively; the gelatin antistress layers of material A contained no cobalt (II) compound.

Strips of the five materials were then stored for 36 hours in an atmosphere of 57° C. and 34% relative humidity and other strips of said materials were stored for 1 week in said atmosphere.

The stored material strips as well as strips of the freshly prepared materials were exposed and developed for 8 minutes at 20° C. in a developing bath having the same composition as that of Example 1.

After the treatment in a stop bath, rinsing and fixing of the material strips the following sensitometric results were attained.

| Material | Freshly prepared |           |                     | Stored for 36 hrs. at 57° C./34% RH |           |                     | Stored for 7 days at 57° C./34% RH |           |                     |
|----------|------------------|-----------|---------------------|-------------------------------------|-----------|---------------------|------------------------------------|-----------|---------------------|
|          | Fog              | Gradation | Rel. speed, percent | Fog                                 | Gradation | Rel. speed, percent | Fog                                | Gradation | Rel. speed, percent |
| A        | 0.02             | 2.8       | 100                 | 0.07                                | 2.8       | 126                 | 0.18                               | 2.8       | 115                 |
| B        | 0.02             | 3.1       | 91                  | 0.03                                | 3.0       | 95                  | 0.05                               | 3.0       | 100                 |
| C        | 0.07             | 3.1       | 81                  | 0.15                                | 2.8       | 79                  | 0.10                               | 3.0       | 85                  |
| D        | 0.09             | 2.5       | 97                  | 0.37                                | 2.3       | 74                  | 0.30                               | 2.9       | 135                 |
| E        | 0.10             | 2.9       | 76                  | 0.09                                | 3.0       | 76                  | 0.06                               | 3.1       | 100                 |

From these results it appears that the cobalt (II) chelates of the invention have a markedly better anti-fogging action than the known cobalt (II) compounds, without giving rise to an appreciable desensitization. Cobalt (II) chloride has also a good fog-inhibiting action but has a higher desensitizing effect.

### EXAMPLE 4

Example 3 was repeated with the difference, however, that the antistress layers of materials D and E comprised, in lieu of the mentioned cobalt (II) salts, equivalent amounts per sq. m. of ethylene diamine tetraacetic acid sodium salt (EDTA Na-salt) and of an aqueous solution of cobalt (II) sulphate and EDTA-Na-salt respectively.

The following sensitometric results were obtained with freshly prepared materials and materials stored for 36 hours in an atmosphere of 57° C. and 34% relative humidity.

| Material | Freshly prepared |           |                         | Stored for 36 hours at 57° C./34% RH |           |                         |
|----------|------------------|-----------|-------------------------|--------------------------------------|-----------|-------------------------|
|          | Fog              | Gradation | Relative speed, percent | Fog                                  | Gradation | Relative speed, percent |
| A        | 0.04             | 3.0       | 100                     | 0.08                                 | 2.8       | 123                     |
| B        | 0.04             | 3.1       | 89                      | 0.04                                 | 3.0       | 100                     |
| C        | 0.06             | 2.9       | 80                      | 0.10                                 | 3.0       | 85                      |
| D        | 0.05             | 3.1       | 102                     | 0.24                                 | 2.7       | 135                     |
| E        | 0.04             | 3.4       | 89                      | 0.04                                 | 3.1       | 100                     |

From these results it appears that the addition of the cobalt (II) chelate from a solution of cobalt (II) sulfate and ethylene diamine tetraacetic acid sodium salt (material E), has the same favorable fog-inhibiting effect as the addition as such of the cobalt (II) chelate of compound 1 disodium salt (material B). The better fog-inhibiting effect of the cobalt (II) chelates as compared with known cobalt (II) compounds is even the more surprising in view of the fog produced in materials C and D where cobalt (II) sulfate and EDTA-Na-salt are used alone.

Analogous tests as described in the above Examples 1 to 4 were carried out with the cobalt (II) chelates of compounds 4, 5, 8, 9 and 13. The same favorable stabilizing and fog-inhibiting effects were obtained.

### EXAMPLE 5

A gelatino silver bromoiodide emulsion as described in Example 1 was divided into 2 aliquot portions.

Each of the two emulsion portions was coated on both sides of a subbed cellulose triacetate support, in such a way that on both sides an amount of silver halide equivalent to 8 g. per sq. m. of silver nitrate was present, and dried. The emulsion layers of the two materials A and B were then overcoated with a gelatin antistress layer, the antistress layers of material B containing 0.07 g. per sq. m. of the manganese (II) chelate of compound 1 disodium salt.

Strips of the two materials were stored for 36 hours in an atmosphere of 57° C. and 34% relative humidity.

The stored material strips as well as strips of the freshly prepared materials were exposed and developed for 8 minutes at 20° C. in a developing bath as described in Example 1.

After the treatment in a stop bath, rinsing and fixing of the material strips the following sensitometric results were attained.

| Material | Freshly prepared |           |                         | Stored for 36 hours at 57° C./34% RH |           |                         |
|----------|------------------|-----------|-------------------------|--------------------------------------|-----------|-------------------------|
|          | Fog              | Gradation | Relative speed, percent | Fog                                  | Gradation | Relative speed, percent |
| A        | 0.11             | 3.11      | 100                     | 0.18                                 | 2.91      | 115                     |
| B        | 0.10             | 3.25      | 105                     | 0.11                                 | 3.07      | 123                     |

Analogous tests, as described in the above Example 5, were carried out with the manganese (II) chelates of compounds 4, 5, 8, 9 and 13. The same favorable stabilizing and fog-inhibiting effects were obtained.

We claim:

1. Photographic light-sensitive silver halide emulsion comprising in said emulsion at least one cobalt (II) or

manganese (II) chelate of a (poly)amino-(poly)carboxylic acid in acid form or in the form of a water-soluble salt wherein said (poly)amino-(poly)carboxylic acid corresponds to the following general formula:



wherein:

10 L stands for alkylene including substituted alkylene and alkylene interrupted by one or more hetero atoms or cycloalkylene including substituted cycloalkylene,  
x represents 0, 1, or 2,

15 R stands for lower alkylene including substituted lower alkylene, and

each of R<sub>1</sub> and R<sub>2</sub> (the same or different) stands for hydrogen, lower alkyl including substituted lower alkyl, aralkyl including substituted aralkyl or aryl including substituted aryl.

20 2. Photographic light-sensitive silver halide emulsion according to claim 1, wherein said cobalt (II) or manganese (II) chelate is present in an amount of from 0.1 g. to 20 g. per mole of silver halide.

25 3. Photographic light-sensitive silver halide emulsion according to claim 1, wherein said emulsion also comprises a stabilizer of the hydroxytriazolo-pyrimidine type.

4. Photographic light-sensitizer silver halide emulsion according to claim 1, wherein the emulsion is a gelatino silver halide emulsion.

30 5. Photographic light-sensitive silver halide material comprising in a gelatin anti-stress layer coated over a silver halide emulsion layer at least one cobalt (II) or manganese (II) chelate of a poly(amino)-(poly)carboxylic acid in acid form or in the form of a water-soluble salt wherein said (poly)amino-(poly)carboxylic acid corresponds to the following general formula:



wherein:

35 L stands for alkylene including substituted alkylene and alkylene interrupted by one or more hetero atoms or cycloalkylene including substituted cycloalkylene,  
x represents 0, 1, or 2,

40 R stands for lower alkylene including substituted lower alkylene, and

each of R<sub>1</sub> and R<sub>2</sub> (the same or different) stands for hydrogen, lower alkyl including substituted lower alkyl, aralkyl including substituted aralkyl or aryl including substituted aryl.

45 6. Photographic material according to claim 5, wherein said cobalt (II) or manganese (II) chelate is present in an amount of from 10 mg. to 1 g. per sq. m. of gelatin anti-stress layer.

7. A process of stabilizing photographic light-sensitive silver halide emulsions, which process comprises exposing to light and developing the light-sensitive silver halide emulsion containing at least one cobalt (II) or manganese (II) chelate of a (poly)amino-(poly)carboxylic acid in acid form or in the form of a water-soluble salt, said (poly)amino-(poly)carboxylic acid having the general formula:



wherein:

20 L stands for alkylene including substituted alkylene and alkylene interrupted by one or more hetero atoms or cycloalkylene including substituted cycloalkylene,  
x represents 0, 1, or 2,

25 R stands for lower alkylene including substituted lower alkylene, and

30 each of R<sub>1</sub> and R<sub>2</sub> (the same or different) stands for hydrogen, lower alkyl including substituted lower alkyl, aralkyl including substituted aralkyl or aryl including substituted aryl.

35 8. A process according to claim 7 wherein said emulsion also contains a stabilizer of the hydroxytriazolo-pyrimidine type.

#### References Cited

##### UNITED STATES PATENTS

2,666,700 1/1954 Baldsiefen ----- 96—107  
2,910,359 10/1959 Maffet ----- 96—110X

45 NORMAN G. TORCHIN, Primary Examiner

J. D. WINKELMAN, Assistant Examiner